

No. 857,886.

PATENTED JUNE 25, 1907.

J. F. MILLER.

METHOD OF LINING TANKS FOR ELECTROLYTIC WORK.

APPLICATION FILED FEB. 6, 1906.

*Fig. 1*



*Fig. 2*



Witnessed

*Raphael Miller*  
*S. S. Dunham*

*J. F. Miller, Inventor*

By his Attorneys  
*Kerr, Page & Cooper.*

# UNITED STATES PATENT OFFICE.

JOHN F. MILLER, OF TRAIL, BRITISH COLUMBIA, CANADA.

## METHOD OF LINING TANKS FOR ELECTROLYTIC WORK.

No. 857,886.

Specification of Letters Patent.

Patented June 25, 1907.

Application filed February 6, 1906. Serial No. 299,691.

*To all whom it may concern:*

Be it known that I, JOHN F. MILLER, a citizen of the United States, residing at Trail, British Columbia, Canada, have invented a 5 certain new and useful Method of Lining Tanks for Electrolytic Work, of which the following is a specification, reference being had to the drawing accompanying and forming part of the same.

10 In the use of wooden tanks or cells for containing the electrolyte in the electrolytic refining of metals considerable difficulty has been experienced in fully protecting the wood from the chemical action of the electrolyte. This is particularly the case with so-called "built up" tanks, that is, tanks constructed of sections united by tie rods or bolts. In such tanks the joints between sections, and also at the angles of the sides, 15 bottom, and ends, are specially liable to be the seat of injury from the electrolyte, resulting in leaks as well as contamination of the electrolyte by the compounds produced by the action of the electrolyte on the wood.

20 Asphaltum, which is unattacked by even powerfully corrosive electrolytes, such for example as are used in the refining of lead by the Betts process, described in Reissued Letters Patent of the United States No. 12,301, 25 dated Jan. 3, 1905, has been commonly used to coat the interior of the tanks, but even asphaltum, as heretofore applied, is not sufficient protection to the joints. The asphaltum must of course be applied while in the 30 molten state, but this is liable to result in bubbles or flows, which may permit the electrolyte or the gases produced therein to penetrate to the wood. I have therefore been led to devise my present invention, which is 35 a method of lining electrolytic tanks, with more particular reference to the joints between the sections composing the same.

40 The nature of the invention will be more readily understood from a somewhat detailed description of the manner in which I prefer to employ it.

45 In the annexed drawing, Figure 1 is a detail sectional view showing a joint between sections of the tank, and showing also the result of the first step of my method. Fig. 2 is a similar section showing the joint completed.

50 The invention is intended more particularly for "built up" tanks of the type shown in my co-pending application filed of even date herewith, in which the joints between

sections and at the angles of the tank are grooved. The preferred form of groove is shown in the annexed drawing. Therein, *a* and *b* indicate contiguous sections from a 50 side, an end, the bottom, or partition of the tank. Each edge is provided with an undercut rabbet, so that when the two are placed together the resulting groove *c* will be wider at its bottom than at its top, as shown. 55

The asphaltum used for the lining must of course have a melting point somewhat higher, say 20° or more, than the temperature at which the electrolyte is to be used. When the asphaltum has been heated to the 70 proper degree of fluidity it is flowed into the groove to a depth say of about one eighth of an inch. While this layer is still warm it is heated, in the groove, in any suitable way, as by passing over it the flame of a gasoline 75 lamp or paint brazier. This heating is kept up until the layer is so liquid that all bubbles or other flows will be eradicated and the asphaltum thus rendered entirely homogeneous. More asphaltum is now run into 80 the groove, immediately or after the first layer has been allowed to cool to a semi-liquid or solid consistency, and the second layer, thus formed, is heated as the first. This operation is repeated until the groove is 85 full of asphaltum free from bubbles or other imperfections and entirely homogeneous throughout. Each joint is treated as described, whereupon the entire surface is flowed with asphaltum to a depth of an 90 eighth of an inch or so. This layer is heated in the manner described in the case of the grooves, more asphaltum is flowed on and heated, and so on until the coating reaches the desired thickness. The result is shown 95 in Fig. 2. This method produces a lining or coating which gives perfect protection to the underlying wood, and the extra thickness at the joints eliminates the trouble due to leaks commonly met with in tanks lined by the 100 methods heretofore in use.

As already stated, asphaltum is a very effective material for the lining, but it is to be understood that my method is not limited to the use of asphaltum. For example, paraffin may be used, or any other substance which will sufficiently resist the chemical action of the particular electrolyte which the tank is to contain.

Having now fully described my invention, 110 what I claim is:

1. The method of coating the interior of an

electrolytic tank, which consists in flowing upon the inner surface of the tank asphaltum liquefied by heat; passing a flame over the layer of asphaltum thus formed, to expel 5 bubbles or other imperfections therefrom; flowing a second layer upon the first, and passing a flame over the same as described; and repeating these steps until a coating of the desired thickness is obtained; as set 10 forth.

2. The method of coating the interior of an electrolytic tank composed of sections the joints between which are formed with grooves in the inner surface of the tank, 15 which consists in depositing a layer of resistant material in the groove, treating the layer to eradicate imperfections therein and render it homogeneous, and repeating these steps until the coating in the grooves is thick 20 as desired; and finally depositing resistant material over the entire inner surface of the tank; as set forth.

3. The method of coating the interior of an electrolytic tank composed of sections the 25 joints between which are formed with grooves in the inner surface of the tank,

which consists in flowing into the grooves layers of resistant material liquefied by heat; each layer being re-heated, in the groove, to expel bubbles or other imperfections, and repeating these steps until the coating in the grooves is thick as desired; then flowing 30 resistant material over the entire inner surface of the tank; heating the layer thus formed to expel bubbles or other imperfections, repeating 35 these steps until the surface coating is thick as desired, as set forth.

4. The method of sealing the joints of an electrolytic tank composed of sections, said joints being formed with grooves in the inner 40 surface of the tank, which consists in flowing melted asphaltum into the groove to form a layer; passing a flame over the layer to heat the same, and thereby expel bubbles or other imperfections therefrom; and repeating these 45 steps as often as may be necessary to produce a deposit of the desired thickness in the groove; as set forth.

JOHN F. MILLER.

Witnesses:

J. M. STRACHAN,  
LEWIS MASSON.